# EUROPEAN PATENT SPECIFICATION

(11) **EP 3 281 720 B1**
(45) Date of publication and mention of the grant of the patent: **02.09.2020**
(21) Application number: 16776475.2
(22) Date of filing: 31.03.2016
(51) Int. Cl.: B21J 13/02, B21J 5/00, B21K 3/04, B21J 7/14, B21J 9/06, B21J 1/04

(54) **HOT FORGING DIE AND HOT FORGING METHOD**
WARMSCHMIEDEGESENK UND WARMSCHMIEDEVERFAHREN
MATRICE DE FORGEAGE À CHAUD ET PROCÉDÉ DE FORGEAGE À CHAUD

(30) Priority: 06.04.2015 JP 2015077338
(43) Date of publication of application: 14.02.2018
(73) Proprietor: Hitachi Metals, Ltd., Tokyo 108-8224 (JP)
(72) Inventor: MITSUNAGA, Hisashi, Yasugi-shi Shimane 692-8601 (JP); FUKUI, Tsuyoshi, Yasugi-shi Shimane 692-8601 (JP); TERAMAE, Toshiya, Yasugi-shi Shimane 692-8601 (JP); NONOMURA, Toshiaki, Yasugi-shi Shimane 692-8601 (JP); MATSUMOTO, Hideki, Yasugi-shi Shimane 692-8601 (JP); SHIMOHIRA, Eiji, Yasugi-shi Shimane 692-8601 (JP); KOHIKI, Satoshi, Yasugi-shi Shimane 692-8601 (JP)
(74) Representative: Reitstötter Kinzebach
(86) International application number: PCT/JP2016/060733
(87) International publication number: WO 2016/163308

(56) References cited:
- EP-A1- 2 149 411
- JP-A- S 535 056
- JP-A- S 561 236
- JP-A- H07 185 725
- JP-A- S55 136 535
- JP-A- S60 250 843
- JP-B2- 3 208 818
- US-A- 611 574
- US-A- 3 893 328
- US-A1- 2004 139 781

## Description

### Technical Field

The present invention relates to a hot forging die and a hot forging method.

### Background Art

For example, during the manufacturing of a turbine blade, a hot forging material having a round rod shape is swaged to a desired diameter, and a preform having a desired round rod shape in which the volume of a portion for forming a root portion or a wing portion of a turbine blade is secured is formed by closed die forging such that a turbine blade material having a near net shape is obtained. Regarding the shape of the preform, for example, Fig. 2 of JP-A-63-238942 (PTL 1) shows a preform having a shape in which a portion for forming a root portion is thick (the volume is high) and is gradually tapered toward a tip of a wing portion.

For example, a specific manufacturing method of the preform includes: radially forging a hot forging material having a round rod shape to obtain a long round bar material having a desired diameter; cutting the long round bar material in a predetermined dimension; and forging the cut round bar material into a desired preform shape using a separate open die forging machine.

During closed die forging of a turbine blade, a portion for forming a root portion or a wing portion, or a protrusion called a boss portion may be provided in a wing portion of the turbine blade. In this case, it is important to adjust the volume and the dimension of a preform for a turbine blade. In a case where the adjustment of the volume and the dimension is insufficient, a preform does not become sufficiently thicker in a die face during closed die forging. Therefore, there is a problem in that a part of a turbine blade material having a near net shape is deficient after closed die forging. In addition, a material of a turbine blade is an expensive alloy such as a Ni-based heat-resistant superalloy or a Ti alloy. Therefore, in a case where a problem, such as deficiency of a part of a turbine blade material having a near net shape after closed die forging, occurs, the damage is significant.

Therefore, it is preferable to provide a groove by processing called "necking" during the manufacturing of a preform such that the preform becomes sufficiently thicker in a die face during closed die forging. However, for example, as disclosed in JP-A-60-250843 (PTL 2), a processing groove may be sequentially formed by necking in a material having a round rod shape using a special jig in a press machine.

A forging material after necking is hot-forged again for swaging (hereinafter, referred to as "swaged") using a separate forging machine in order to obtain a predetermined preform shape. JP 3 208818 B2, on which the preamble of claim 1 is based, shows a hot forging die and method for hot-forging a rod shaped forging material by radial forging.

### Citation List

### Patent Literature

[PTL 1] JP-A-63-238942
[PTL 2] JP-A-60-250843

### Summary of Invention

### Technical Problem

As disclosed in PTL 2, in the related art, only a jig for necking is improved, and a hot forging die suitable for swaging which is performed after necking is not disclosed.

Regarding a shape of a pressing portion disclosed in PTL 2, the pressing portion is formed smooth and is not suitable for forming a desired groove in a difficult-to-work material. Further, a groove formed by necking has a small width and is vertically deep. In a case where a groove is formed in a direction perpendicular to a depth direction of a forging material, there is a problem in that an overlap defect occurs during hot forging in which the forging material is swaged to the length of a turbine blade.

An object of the present invention is to provide a hot forging die and a hot forging method, in which even a difficult-to-work material used for a turbine blade can be easily swaged using a radial forging machine.

### Solution to Problem

The present invention has been made in consideration of the above-described circumstances.

That is, according to the present invention, there is provided a hot forging die for hot-forging a rod shaped forging material by radial forging, according to claim 1.

In the hot forging die, it is preferable that the width of the halved pressing portion gradually increases in a direction from the rough processing portion to the finishing portion.

In the hot forging die, it is more preferable that the width of the finishing portion is wider than the width of the rough processing portion by 10 mm or more.

In addition, the finishing portion may include a concave portion that divides a pressing surface of the finishing portion into two or more areas.

It is preferable that the hot forging die is used for swaging the forging material.

In addition, according to the present invention, there is provided a hot forging method for hot-forging a rod shaped forging material by radial forging, according to claim 6.

In the hot forging method, it is preferable that the rod shaped forging material is formed of a Ni-based heat-resistant superalloy or a Ti alloy.

The hot forging method according to the present invention is suitable for manufacturing a preform for a turbine blade.

### Advantageous Effects of Invention

According to the present invention, even a difficult-to-work material used for a turbine blade or the like can be easily swaged using a radial forging machine.

### Brief Description of Drawings

Fig. 1 is a schematic diagram showing an example of a hot forging die according to the present invention.
Fig. 2 is a schematic diagram showing an example of a necking portion.
Fig. 3 is a schematic diagram showing an example of the necking portion.
Fig. 4 is a schematic diagram showing a radial forging machine.
Fig. 5 is a schematic diagram showing an example of a shape of a preform.
Fig. 6 is a schematic diagram showing an example of the hot forging die according to the present invention.
Fig. 7 is a schematic diagram showing an example of a portion that presses a forging material when the hot forging die according to the present invention is used for hot forging.
Fig. 8 is a schematic diagram showing an example of a portion that presses a forging material when the hot forging die according to the present invention is used for hot forging.
Fig. 9 is a schematic diagram showing an example of the hot forging die according to the present invention.

### Description of Embodiments

The greatest feature of the present invention is a hot forging die having a novel shape and a hot forging method using the hot forging die which are applicable to formation of a preform for a large turbine blade using a radial forging machine. Hereinafter, a hot forging die used in the present invention will be described.

Fig. 1 shows a schematic side view showing a hot forging die 1 according to the present invention, a cross-sectional view (cross-sectional view D-D) showing a finishing portion of the hot forging die 1, a cross-sectional view (cross-sectional view F-F) showing a rough processing portion of the hot forging die 1, and a cross-sectional view (cross-sectional view E-E) showing a space between the finishing portion and the rough processing portion. In the present invention, a radial forging machine that presses a forging material in two directions opposite to each other is used. In Fig. 1, the width of a smooth surface of a pressing portion (the width in a longitudinal direction of a forging material) gradually increases from a width W1 of a position shown in the cross-sectional view F-F to a width W2 of a position shown in the cross-sectional view E-E. A width W3 of the smooth surface of the pressing portion in a region from the width W2 of the position shown in the cross-sectional view E-E to a position (bottom) shown in the cross-sectional view D-D is substantially the same. "The finishing portion" described in the present invention refers to a portion having the same width which includes the position (bottom) shown in the cross-sectional view D-D. In the finishing portion, a portion that presses the forging material may have a smooth surface which is formed to be concave as shown in Fig. 1, and a concave portion may be provided in a part of the portion that presses the forging material as described below.

Two hot forging dies 1 shown in Fig. 1 are set as a pair. For example, as shown in Fig. 4, the two hot forging dies are facing each other such that a forging material 21 is interposed therebetween, and the pair of two hot forging dies 1 cooperate together for swaging. The portion that swages the forging material includes halved pressing portions 2 between which the forging material (not shown in Fig. 1) is interposed. The forging material is interposed between the halved pressing portions and pressed. The forging material is held and intermittently rotated by a holding mechanism included in a radial forging machine.

As shown in the schematic side view of Fig. 1, each of the halved pressing portions 2 includes a plurality of continuous surfaces (a pressing surface as a working surface, and inclined side surfaces that are provided on opposite sides of the pressing surface), and that form a continuous convex shape so as to surround the forging material. Since the pressing portions has halved shape, the forging material can be interposed between the pressing portions of the two hot forging dies that cooperate together. In addition, "the shape which is continuous so as to surround the forging material" refers to a shape in which the periphery of the forging material 21 is surrounded by the rough processing portions and the finishing portions as shown in Fig. 4. The halved pressing portion 2 is formed such that a smooth surface has a concave shape, and the pressing portion has an arc shape when seen from the side (in the schematic side view of Fig. 1). The halved pressing portion 2 includes a finishing portion 4 and rough processing portions 3. The finishing portion 4 is formed around the concave (arc-shaped) bottom, and the rough processing portions 3 are formed on each of both sides (opposite end sides of the concave (arc-shaped) portion) of the finishing portion. The distance between the rough processing portions increases in a direction from the bottom of the finishing portion 4 to the end portions of the opposite rough processing portions 3. When the two hot forging dies press the forging material, the forging material can be pressed in a continuous convex shape. In a case where the forging material is hot-forged by the hot forging die 1 having the above-described shape, the convex rough processing portions formed in the hot forging die comes into contact with the forging material first such that the forging material can be sequentially formed in a predetermined dimension. Therefore, "the convex shape" described in the present invention refers to a shape when seen from the direction of the respective cross-sectional views. That is, the cross-section refers to a cross-section seen from a direction perpendicular to the longitudinal direction of the forging material. The pressing portion (working surface) that is formed to be convex and swages the forging material has a structure in which a smooth surface which is formed to be a concave shape. Therefore, in the present invention, the above-described pressing portion (working surface) will also be referred to as "smooth pressing portion".

In addition, each of the halved pressing portions 2 includes: rough processing portions 3; and a smooth finishing portion 4 in which a width of the pressing portion (width in the longitudinal direction of the forging material) is wider than that of the rough processing portion 3. The reason for this is as follows. In the initial stage of swaging, the contact area is reduced for effective necking such that even a difficult-to-work forging material can be efficiently swaged when the forging of the forging material starts from the rough processing portions. Along with the progress of swaging, the forging material is sequentially pressed toward the finishing portion having a wide width of the pressing portion such that the shape of the forging material is adjusted to a final shape. The pressing portion disclosed in the above-described PTLs 1 and 2 is formed to have the same width. However, it is advantageous to change the contact area particularly when a difficult-to-work material is swaged.

That is, in the present invention, initially, the forging material can be efficiently swaged by the rough processing portion 3 having a small contact area with the forging material. Next, the forging material can be efficiently formed in a final shape by the finishing portion 4 having a wider width of the pressing portion than the rough processing portion 3. Therefore, it is preferable that the width of the pressing portion gradually increases from the width of the pressing portion of the rough processing portion 3 to the width of the pressing portion (finishing surface) of the finishing portion 4 having a wider width than the rough processing portion.

The actual pressing portion may be repaired, for example, by build-up welding, and then the shape may be manually machined. Therefore, the shape of the actual pressing portion is not necessarily a smooth shape having substantially no irregularity. Therefore, "the smooth shape" described in the present invention only has to be a smooth shape having no significantly irregularity which has a margin of error generated by build-up welding or machining. The shape may be determined from an approximate shape. In addition, the hot forging die according to the present invention includes the halved pressing portions. Therefore, the working surface is curved so as to surround the forging material.

It is preferable that the width of the pressing portion of the finishing portion 4 according to the present invention (the width in the longitudinal direction of the forging material) is wider than the width of the pressing portion of the rough processing portion 3 by 10 mm or more. The reason for this is as follows. By increasing a difference between the contact areas to increase the amount of processing in the initial stage of swaging, the forging material can be accurately finished into a predetermined shape in the final stage of swaging. In a case where a difference in width between the finishing portion and the rough processing portion is less than 10 mm, the effect cannot be sufficiently obtained. Therefore, the difference is adjusted to be 10 mm or more. The difference is preferably 15 mm or more.

It is preferable that an inclination θ of a flank formed in a continuous portion leading to the finishing portion 4 is preferably 15° to 35°. The flank is a surface which is formed on a side where the forging material is supplied. The flank is transferred to the forging material at a hot forging and the transferred portion (A portion in Fig. 6) is forged at the forging. As a result, the occurrence of an overlap defect in the forging material can be prevented. In Fig. 1, the flanks are formed on both sides of the finishing portion. In a case where the hot forging die having the above-described structure is used, the forging material can be swaged while reciprocating the forging material. For example, in a case where the forging material is swaged in only one direction, the flank may be formed only one side where the forging material is supplied as shown in Fig. 6.

For example, in a case where a preform for a turbine blade is formed, processing called necking is performed before swaging the forging material. The hot forging die 11 used for necking includes a necking portion 7 that forms a processing groove. A pressing portion for necking provided in the necking portion 7 is formed such that includes a gradual change portion having an arc-shaped cross-section of the pressing portion in which the curvature radius of the arc-shaped cross-section of the pressing portion gradually increases from the rough processing portion (cross-sections C-C and G-G) to the finishing portion (cross-sections A-A, B-B, E-E, and F-F) as shown in Figs. 2 and 3. The necking portion 7 for necking includes a pair of halved pressing portions 12 between which the forging material is interposed, in which each of the halved pressing portions 12 has a convex portion having a substantially semicircular cross-section, the convex portion being continuous so as to surround the forging material, and each of the halved pressing portions 12 includes a rough processing portion 13 having a substantially semicircular cross-section and a finishing portion 14. In addition, each of the halved pressing portions includes the rough processing portion and the convex finishing portion having a convex portion having a larger curvature radius than the rough processing portion. The curvature radius of the cross-section of the halved pressing portion from a position shown in the B-B cross-section to a position shown in the A-A cross-section and the curvature radius of the cross-section of the halved pressing portion from a position shown in the F-F cross-section to a position shown in the E-E cross-section is identical.

The basic configuration is the same as that of the hot forging die suitable for swaging. Likewise, two hot forging dies 11 for necking are set as a pair. During the necking of the forging material, the forging material is held and rotated by a holding mechanism included in a radial forging machine such that the pair of hot forging dies 11 for necking cooperate together to form a predetermined groove in the forging material (not shown).

In addition, in the hot forging die for necking, as shown in Fig. 3, a plurality of pressing portions 12 for necking may be formed in the longitudinal direction of the forging material. The reason for this is as follows. In a case where two or more processing grooves are formed by necking, it is advantageous to form a plurality of pressing portions 12 for necking in one die from the viewpoint of productivity. In particular, an alloy material used for a turbine blade is a difficult-to-work material. Therefore, it is preferable that forging is finished within the shortest possible time in a temperature range where hot forging is possible. The simultaneous formation of a plurality of grooves by necking is effective in a portion for forming a boss portion which is provided in a wing portion of a turbine blade.

The simultaneous formation of a plurality of grooves by necking can be realized by using a radial forging machine in combination with the hot forging die according to the present invention in which the contact area of the pressing portion gradually increases from a small area to a large area.

In the hot forging die having a structure shown in Figs. 2 and 3, similarly, the finishing portion is a portion (ranging from a position shown in the cross-sectional view F-F to a position shown in the cross-sectional view E-E and ranging from a position shown in the cross-sectional view B-B to a position shown in the cross-sectional view A-A) having an identical curvature radius which includes a position (bottom) shown in the cross-sectional view E-E and the cross-sectional view A-A.

Next, a hot forging method of forming a preform for 50-inch turbine blade using the hot forging die according to the present invention will be described as an example.

Fig. 4 is a schematic diagram showing an example of a radial forging machine. The hot forging die 11 shown in Fig. 2 or 3 is attached to the radial forging machine. Each of the hot forging dies 11 are provided on each of opposite surfaces to the forging material such that the forging material 21 is interposed between the hot forging dies 11. In Fig. 4, the forging material 21 is held in the radial forging machine. The forging material is heated to a predetermined hot forging temperature in a heating furnace (not shown) and is attached to the radial forging machine.

The heating temperature varies depending on the material of the forging material. For example, in a case where the material of the forging material is a Ni-based heat-resistant superalloy, the heating temperature is 950°C to 1150°C. In a case where the material of the forging material is a Ti alloy, the heating temperature is 800°C to 1000°C. In addition, in a case where the material of the forging material is a precipitation hardening stainless steel, the heating temperature is 900°C to 1200°C. In addition, the shape of the forging material is a rod shape. The rod shaped forging material only has to be adjusted to a predetermined shape using a forging machine or a press machine. In a case where the forging material has a round rod shape, it is preferable that the diameter of the forging material is the same as the distance of the rough processing portions of the hot forging die 11 for necking.

Among the above-described forging materials, the forging material having a predetermined round rod shape is attached to the radial forging machine.

During the hot forging, the forging material is necked by rotating the heated forging material 21 and concurrently pressing the forging material using each of the halved pressing portions of the pair of two hot forging dies 11 which are facing each other. The shape of the hot forging die for necking is as shown in Fig. 2 or 3. During necking, hot forging starts from the rough processing portions 13 of the hot forging die 11. The hot forging die according to the present invention has a shape in which the distance between the rough processing portions increases in a direction from the finishing portion 14 to the rough processing portions 13 and in which, when the two hot forging dies press the forging material, the forging material can be pressed in a continuous substantially semicircular convex shape. In addition, during initial necking, the forging material rotates at the same position (does not move in the longitudinal direction of the forging material).

Examples of a necking method include two methods. As a first method, a method in which the shape after completion of necking is emphasized will be described first.

In a case where hot forging starts from two directions opposite to each other, as shown in Fig. 7(A), predetermined positions of the forging material start to be pressed by the rough processing portions 13 first. Contact (forging) positions between the forging material 21 and the hot forging die during rough processing are indicated by arrows. As a result, the forging material is hot-forged in the two directions opposite to each other and, in the initial stage of forging, starts to be pressed by the rough processing portions formed in the two hot forging dies that cooperate together to forge the forging material. Thus, the number of positions where the forging material is pressed at the start of forging is four. In a case where necking starts at the four positions at the same time, the contact area is small, and thus a groove can be efficiently formed. By sequentially hot-forging the forging material toward the finishing portions, the shape of the forging material is adjusted to a predetermined shape in the finishing portions that are formed in the pair of hot forging dies. In the final stage of finishing, as shown in Fig. 7(B), the number of positions where the forging material 21 is pressed during hot forging in the bottoms of the finishing portions is two. That is, in the initial stage of necking, the four positions are forged (necked) using the pair of hot forging dies. During the adjustment of a final shape, the two positions are forged using the pair of hot forging dies. As a result, the shape of the forging material can be adjusted. In addition, the forging material can be efficiently formed in a final shape in the convex finishing portions 14 having a larger curvature radius than the rough processing portions. Further, the final shape of the forging material can be adjusted to the bottom shape of the finishing portion indicated by an arrow. Therefore, this method is suitable in a case where the final finished shape is emphasized.

A second method is a method which is applicable to a case where the processing time is short.

In a case where hot forging starts from two directions opposite to each other, as shown in Fig. 8(A), predetermined positions of the forging material start to be pressed by the rough processing portions 13 first. Contact (forging) positions between the forging material 21 and the hot forging die during rough processing are indicated by arrows. As a result, the forging material is hot-forged in the two directions opposite to each other and, in the initial stage of forging, starts to be pressed by the rough processing portions formed in the two hot forging dies that cooperate together to forge the forging material. Thus, the number of positions where the forging material is pressed at the start of forging is four. In a case where necking starts at the four positions at the same time, the contact area is small, and thus a groove can be efficiently formed. By sequentially hot-forging the forging material toward the finishing portions, the shape of the forging material is adjusted to a predetermined shape in the finishing portions 14 that are formed in the pair of hot forging dies.

As described above, in a region from the position shown in the cross-sectional view B-B to a position (bottom) shown in the cross-sectional view A-A, the curvature radius is substantially the same. Therefore, finishing is not performed in the bottoms of the finishing portions and can be finished in a state where the number of positions where the hot forging material is pressed during finishing is four as shown in Fig. 8(B). Even in this case, the forging material can be efficiently formed in a final shape in the convex finishing portion 14 having a larger curvature radius than the rough processing portion. In addition, since the number of positions where the hot forging material is pressed is four, necking can be finished within a short period of time. Thus, this method is suitable in a case where it is desired that the forging time is short.

In the method in which the forging time is emphasized, it is important to adjust the curvature radius (the curvature radius when seen from a direction perpendicular to the longitudinal direction of the forging material shown in Fig. 8) of the bottom (position shown in the cross-sectional view A-A) of the finishing portion to be less than the curvature radius of the diameter after necking. In this case, it is preferable that the bottom of the finishing portion is curved in order to avoid excessive stress concentration during hot forging.

Once necking is completed, the hot forging die 11 is replaced with the hot forging die 1 including a pressing portion for swaging. When the hot forging dies are replaced, the forging material is reheated to a predetermined forging temperature.

The replaced hot forging die 1 includes a swaging portion 5 including the pressing portion for swaging that swages the forging material.

The pressing portion for swaging has a shape shown in Fig. 1. When the hot forging die including the pressing portion for swaging is seen from the longitudinal direction of the forging material, the shape of the pressing portion is the same as that of the hot forging die 11 for necking shown in Fig. 7(A). Therefore, in a case where hot forging starts from two directions opposite to each other, predetermined positions of the forging material start to be pressed by the rough processing portions 3 first. As a result, the forging material is hot-forged in the two directions opposite to each other and, in the initial stage of swaging (forging), starts to be pressed by the rough processing portions formed in the two (the pair of) hot forging dies that cooperate together to forge the forging material. Thus, the number of positions where the forging material is pressed at the start of forging is four. In a case where swaging starts at the four positions at the same time, the contact area is small, and thus the forging material can be efficiently swaged. The forging material is sequentially moved in the longitudinal direction of the forging material while being intermittently rotated by the radial forging machine, and then is sequentially hot-forged toward the finishing portions. As a result, the shape of the forging material is adjusted to a predetermined shape in the finishing portions that are formed in the pair of hot forging dies. That is, in the final stage of finishing, as shown in Fig. 7(B), the number of positions where the forging material is pressed during hot forging in the finishing portions 14 is two. The method of adjusting the final shape to the bottom shape of the finishing portion is suitable in a case where the final finished shape is emphasized.

In addition, in order to reduce the hot forging time during hot forging using the pressing portion for swaging, the number of positions where the hot forging material is pressed from the initial stage to the final stage of hot forging is adjusted to four as shown in Fig. 8. As a result, the forging material can be swaged within a short period of time.

In the present invention, the hot forging die including the pressing portion for swaging can be made to have a shape shown in Fig. 9. In the hot forging die 1 shown in Fig. 9, a concave portion 6 is formed in a region from the bottom in the width of the finishing portion 4 (the width in the longitudinal direction of the forging material) to the rough processing portion. Due to the concave portion 6, the pressing surface of the finishing portion is divided into two areas. By forming one or more concave portions in the width (W3) of the finishing portion 4 to divide the pressing surface of the finishing portion into two or more areas, the forging material can be more reliably prevented from being bent during swaging. In a case where the forging material is hot-forged using the hot forging die shown in Fig. 9, the final stage of forging is performed in the bottom of the finishing portion shown in the cross-sectional view A-A. When the forging material is pressed, there are two portions including: a pressed portion that is pressed by the finishing portion; and a portion that is not pressed by the finishing portion and is adjacent to the portion pressed by the finishing portion. A part of the pressed portion flows to the non-pressed portion such that the cross-section of the forging material is slightly elliptical. The elliptical forging material is likely to be bent during forging. However, in the structure of the hot forging die shown in Fig. 9, the pressing surface (finishing portion) is divided by the concave portion. Therefore, the forging material is intermittently rotated by radial forging in the initial pressing portion and is finished in the next pressing surface. At this time, four portions in total are pressed in the structure shown in Fig. 9. Therefore, as described above, an elliptical shape and a bent shape can be corrected in the pressing surface. By forming the concave portion at positions including the bottom of the finishing portion (the position in contact with the straight line A-A in Fig. 9), the effect of preventing bending can be exhibited as much as possible.

This way, the forging material can be continuously hot-forged into a predetermined preform shape by using the same radial forging machine not only for necking but also for swaging. Therefore, unlike the related art, it is not necessary to perform swaging using a separate forging machine after using a jig for necking. That is, a troublesome process can be reduced. Thus, although the number of times of reheating is reduced, a preform for a high-accuracy turbine blade can be manufactured.

According to the present invention, even a difficult-to-work material used for a turbine blade can be easily swaged using a radial forging machine. In addition, according to the novel hot forging method using a radial forging machine, the number of times of reheating a forging material can be significantly reduced, the productivity can be improved, and this method is extremely effective in power saving.

### Examples

### (Example 1)

The hot forging die 11 shown in Fig. 3 was prepared.

The necking portion 7 of the prepared hot forging die 11 for necking includes a pair of halved pressing portions 12 between which the forging material is interposed, in which each of the halved pressing portions 12 has a convex portion having a substantially semicircular cross-section which is continuous so as to surround the forging material 21, and each of the halved pressing portions 12 includes a rough processing portion 13 and a finishing portion 14 having a convex portion having a larger curvature radius than the rough processing portion. The curvature radius of the necking portion 7 gradually changes, in which the curvature radius of the substantially semicircular convex portion of the rough processing portion 13 is 30 mm, and the curvature radius of the substantially semicircular convex portion of the finishing portion 14 is 50 mm.

In addition, regarding the pressing portion for swaging provided in the swaging portion 5 of the hot forging die 1 that swages the forging material 21 after necking, the pressing portion is formed smooth, and the shape thereof is as shown in Fig. 1. The pressing portion for swaging includes a pair of halved pressing portions 2 between which the forging material is interposed, in which each of the halved pressing portions 2 has a substantially semicircular convex shape which is continuous so as to surround the forging material 21, and each of the halved pressing portions 2 includes a substantially flat rough processing portion 3 and a finishing portion 4. The width of the pressing portion for swaging gradually changes, in which the width of the rough processing portion 3 is 50 mm, and the width of the finishing portion 4 is 100 mm. The inclination θ of the flank is 18°. The hot forging die has a shape in which a final shape is emphasized.

The above-described two hot forging dies were set as a pair, and the pair of hot forging dies were attached to a radial forging machine.

A forging material for a 50-inch turbine blade was heated in a heating furnace heated to 950°C. The forging material was formed of a titanium alloy, in which the diameter was φ200 mm and the length was 1100 mm.

The forging material was extracted from the heating furnace and started to be hot-forged in the radial forging machine. The forging material was held by a manipulator.

During the hot forging, the forging material was necked by rotating the heated forging material 21 and concurrently pressing the forging material using each of the halved pressing portions of the pair of two hot forging dies 1 which were facing each other. During initial necking, the forging material was hot-forged into a predetermined shape while rotating the forging material at the same position (not moving in the longitudinal direction of the forging material). As shown in Fig. 3, a plurality of halved pressing portions 12 for necking were formed in one die, and two portions were necked at the same time using this die.

After completion of necking, the hot forging die was replaced with the hot forging die 1 of Fig. 1 including the pressing portion for swaging. At this time, the forging material was extracted from the radial forging machine and was reheated to a predetermined forging temperature. After completion of the replacement with the hot forging die 11 including the pressing portion for swaging, the forging material was attached to the radial forging machine again and was hot-forged using the pressing portion for swaging. The forging material was intermittently rotated by the radial forging machine and was sequentially moved in the longitudinal direction such that the shape thereof was adjusted to a predetermined shape. As a result, the forging material was hot-forged into a preform shape. A preform 22 after hot forging had a shape shown in Fig. 5 which was suitable for forming a root portion, a wing portion, or a boss portion. In the preform after hot forging, a preform such as an overlap defect did not occur.

With the method according to the present invention, even a difficult-to-work material used for a turbine blade or the like can be easily swaged using a radial forging machine. In addition, a forging material can be hot-forged and necked into a predetermined preform shape using a radial forging machine. Therefore, unlike the related art, a troublesome process such as use of a jig for necking can be reduced. Thus, although the number of times of reheating is reduced, a preform for a high-accuracy turbine blade can be manufactured.

### (Example 2)

In Example 2, the effect of the hot forging die shown in Fig. 9 was verified. In the hot forging die shown in Fig. 9, the width of the pressing portion for swaging gradually changes, in which the width of the pressing portion for swaging 5 in the rough processing portion 3 is mm, and the width of the pressing portion for swaging 5 in the finishing portion 4 is 120 mm. A concave portion having a width of 50 mm was formed at the center of the finishing portion, and the number of pressing surfaces in the finishing portion was 2. The width of each of the two divided pressing surfaces was 35 mm. The same hot forging die for necking as in Example 1 was used.

A forging material for a 50-inch turbine blade was heated in a heating furnace heated to 950°C. The forging material was formed of a titanium alloy, in which the diameter was φ200 mm and the length was 1100 mm.

The forging material was extracted from the heating furnace and started to be hot-forged in the radial forging machine. The forging material was held by a manipulator.

During the hot forging, the forging material was necked by rotating the heated forging material 21 and concurrently pressing the forging material using each of the halved pressing portions of the pair of two hot forging dies 11 which were facing each other. During initial necking, the forging material was hot-forged in a predetermined shape while rotating the forging material at the same position (not moving in the longitudinal direction of the forging material). As shown in Fig. 3, a plurality of halved pressing portions 12 for necking were formed in one die, and two portions were necked at the same time using this die.

After completion of necking, the hot forging die was replaced with the hot forging die 1 of Fig. 9 including the pressing portion for swaging. At this time, the forging material was extracted from the radial forging machine and was reheated to a predetermined forging temperature. After completion of the replacement with the hot forging die 1 including the pressing portion for swaging, the forging material was attached to the radial forging machine again and was hot-forged using the pressing portion for swaging. The forging material was intermittently rotated by the radial forging machine and was sequentially moved in the longitudinal direction such that the shape thereof was adjusted to a predetermined shape. As a result, the forging material was hot-forged into a preform shape. Finally, the hot forging die was replaced with the hot forging die 1 shown in Fig. 9, and the forging material was finished using 10-pass radial forging. A preform 22 after hot forging had a shape shown in Fig. 5 which was suitable for forming a root portion, a wing portion, or a boss portion. In the preform after hot forging, a preform such as an overlap defect did not occur. Regarding the bending of the preform having a total length of about 1500 mm, it was verified that bending of about 5 mm was suppressed by comparing the preform obtained in Example 2 to the preform obtained in Example 1.

With the method according to the present invention, even a difficult-to-work material used for a turbine blade or the like can be easily swaged using a radial forging machine. In addition, a forging material can be hot-forged and necked into a predetermined preform shape using a radial forging machine. Therefore, unlike the related art, a troublesome process such as formation of a mark at a necking position can be reduced. Thus, although the number of times of reheating is reduced, a preform for a high-accuracy turbine blade can be manufactured.

## Claims

1. A hot forging die (1) for hot-forging a rod shaped forging material by radial forging, the hot forging die comprising a pair of halved pressing portions (2) for interposing the forging material between the pair of the halved pressing portions (2), each of the halved pressing portions (2) having a smooth surface having a concave shape configured to surround the forging material,
wherein the halved pressing portion includes rough processing portions (3) and a finishing portion (4), and
a width of the finishing portion in a longitudinal direction of the forging material is wider than a width of the rough processing portions,
**characterized in that** the finishing portion (4) is formed around a bottom of the concave shape, and
rough processing portions (3) are formed on each of both sides of the finishing portion (4), on opposite end sides of the concave shape.

2. The hot forging die (1) according to claim 1, wherein the width of the halved pressing portion (2) gradually increases in a direction from the rough processing surface to the finishing surface.

3. The hot forging die (1) according to claim 1 or 2, wherein the width of the finishing portion (4) is wider than the width of the rough processing portion (3) by 10 mm or more.

4. The hot forging die (1) according to any one of claims 1 to 3, wherein the finishing portion (4) includes a concave portion (6) that divides a pressing surface of the finishing portion (4) into two or more areas.

5. The hot forging die (1) according to any one of claims 1 to 4, wherein the hot forging die is a hot forging die for swaging the forging material.

6. A hot forging method for hot-forging a rod shaped forging material by radial forging by using the hot forging die (1) according to any one of claims 1 to 5,
wherein the hot forging method comprising:
a forging material heating step of heating the forging material to a hot forging temperature; and
a hot forging step of swaging the forging material by rotating the heated forging material and concurrently pressing the forging material with the hot forging die (1) at the pair of the halved pressing portions (2) facing each other.

7. The hot forging method according to claim 6, wherein the rod shaped forging material is formed of a Ni-based heat-resistant superalloy or a Ti alloy.

8. The hot forging method according to claim 6 or 7, wherein the forging material is a preform for a turbine blade.

## Patentansprüche

1. Warmschmiedegesenk (1) zum Warmschmieden eines stabförmigen Schmiedematerials durch Radialschmieden, wobei das Warmschmiedegesenk ein Paar von Pressteil-Hälften (2) umfasst, um das Schmiedematerial zwischen das Paar von Pressteil-Hälften (2) einzubringen, jede Pressteil-Hälfte (2) eine glatte Oberfläche mit einer konkaven Form hat, die so ausgebildet ist, dass sie das Schmiedematerial umgibt,
bei dem die Pressteil-Hälfte Grobbearbeitungs-Abschnitte (3) und einen Endbearbeitungs-Abschnitt (4) aufweist, und
die Breite des Endbearbeitungs-Abschnitts in Längsrichtung des Schmiedematerials breiter ist als die Breite der Grobbearbeitungs-Abschnitte,
**dadurch gekennzeichnet, dass** der Endbearbeitungs-Abschnitt (4) an der Unterseite der konkaven Form ausgebildet ist, und
die Grobbearbeitungs-Abschnitte (3) an jeder der beiden Seiten des Endbearbeitungs-Abschnitts (4) an gegenüberliegenden Stirnseiten der konkaven Form ausgebildet sind.

2. Warmschmiedegesenk (1) nach Anspruch 1, bei dem die Breite der Pressteil-Hälfte (2) allmählich in Richtung von der Grobbearbeitungs-Oberfläche zur Endbearbeitungs-Oberfläche zunimmt.

3. Warmschmiedegesenk (1) nach Anspruch 1 oder 2, bei dem die Breite des Endbearbeitungs-Abschnitts (4) mindestens 10 mm größer ist als die Breite des Grobbearbeitungs-Abschnitts (3).

4. Warmschmiedegesenk (1) nach einem der Ansprüche 1 bis 3, bei dem der Endbearbeitungs-Abschnitt (4) einen konkaven Abschnitt (6) enthält, der die Press-Oberfläche des Endbearbeitungs-Abschnitts (4) in zwei oder mehr Bereiche aufteilt.

5. Warmschmiedegesenk (1) nach einem der Ansprüche 1 bis 4, bei dem das Warmschmiedegesenk ein Warmschmiedegesenk zum Gesenkschmieden des Schmiedematerials ist.

6. Warmschmiedeverfahren zum Warmschmieden eines stabförmigen Schmiedematerials durch Radialschmieden unter Verwendung des Warmschmiedegesenks (1) nach einem der Ansprüche 1 bis 5,
wobei das Warmschmiedeverfahren umfasst:
einen Schmiedematerial-Heizschritt zum Erhitzen des Schmiedematerials auf eine Warmschmiedetemperatur; und
einen Warmschmiedeschritt zum Gesenkschmieden des Schmiedematerials durch Rotieren des erhitzten Schmiedematerials und gleichzeitiges Pressen des Schmiedematerials mit dem Warmschmiedegesenk (1) an das Paar der gegenüberliegenden Pressteil-Hälften (2).

7. Warmschmiedeverfahren nach Anspruch 6, bei dem das stabförmige Schmiedematerial aus einer Ni-basierten hitzebeständigen Superlegierung oder einer Ti-Legierung geformt ist.

8. Warmschmiedeverfahren nach einem der Ansprüche 6 oder 7, bei dem das Schmiedematerial eine Vorform für eine Turbinenschaufel ist.

## Revendications

1. Matrice de forgeage à chaud (1) pour le forgeage à chaud d'un matériau de forgeage en forme de barre par forgeage radial, la matrice de forgeage à chaud comprenant une paire de parties de pressage en moitiés (2) pour interposer le matériau de forgeage entre la paire de parties de pressage en moitié (2), chacune des parties de pressage en moitiés (2) ayant une surface lisse ayant une forme concave configurée pour entourer le matériau de forgeage,
dans laquelle la partie de pressage en moitié comporte des parties de traitement rugueuses (3) et une partie de finition (4), et
une largeur de la partie de finition dans une direction longitudinale du matériau de forgeage est plus large qu'une largeur des parties de traitement rugueuses,
**caractérisée en ce que** la partie de finition (4) est formée autour d'un fond de la forme concave, et
des parties de traitement rugueuses (3) sont formées sur chacun des deux côtés de la partie de finition (4), sur des côtés d'extrémité opposés de la forme concave.

2. Matrice de forgeage à chaud (1) selon la revendication 1, dans laquelle la largeur de la partie de pressage en moitié (2) augmente progressivement dans une direction de la surface de traitement rugueuse à la surface de finition.

3. Matrice de forgeage à chaud (1) selon la revendication 1 ou 2, dans laquelle la largeur de la partie de finition (4) est plus large que la largeur de la partie de traitement rugueuse (3) de 10 mm ou plus.

4. Matrice de forgeage à chaud (1) selon l'une quelconque des revendications 1 à 3, dans laquelle la partie de finition (4) comporte une partie concave (6) qui divise une surface de pressage de la partie de finition (4) en au moins deux zones.

5. Matrice de forgeage à chaud (1) selon l'une quelconque des revendications 1 à 4, la matrice de forgeage à chaud étant une matrice de forgeage à chaud destinée à la rétreinte du matériau de forgeage.

6. Procédé de forgeage à chaud pour le forgeage à chaud d'un matériau de forgeage en forme de barre par forgeage radial à l'aide de la matrice de forgeage à chaud (1) selon l'une quelconque des revendications 1 à 5,
le procédé de forgeage à chaud comprenant :
une étape de chauffage de matériau de forgeage consistant à chauffer le matériau de forgeage jusqu'à une température de forgeage à chaud ; et
une étape de forgeage à chaud consistant en une rétreinte du matériau de forgeage par rotation du matériau de forgeage chauffé et pressage simultané du matériau de forgeage avec la matrice de forgeage à chaud (1) au niveau de la paire de parties de pressage en moitiés (2) face à face.

7. Procédé de forgeage à chaud selon la revendication 6, dans lequel le matériau de forgeage en forme de barre est formé d'un superalliage résistant à la chaleur à base de Ni ou d'un alliage de Ti.

8. Procédé de forgeage à chaud selon la revendication 6 ou 7, dans lequel le matériau de forgeage est une préforme pour une aube de turbine.
